

## 1

2,763,583

## PROCESS FOR MANUFACTURING POROUS CAST IRON

Sozo Kawasaki, Minatoku, Tokyo, Japan

No Drawing. Application March 26, 1953,  
Serial No. 344,891

6 Claims. (Cl. 148—21.7)

This invention relates to a method for easily producing cast iron which is excellently permeable by oil and is suitable for use in oilless bearings or the like.

This invention has for its object to increase the porosity of oil permeable cast iron so that it may contain the maximum possible amount of oil, without sacrificing its mechanical strength.

Where it is desired to make a bearing of an oil permeable metallic material made by sintering finely divided material in a forming mold therefor, the porosity of the surface of the product thus obtained tends to be impaired by the subsequent machining operations. This difficulty manifests itself particularly when such metals as copper, tin, etc., are used as the raw material.

It is well known that if a cast iron is repeatedly subjected to annealing, the phenomenon of the expansion of the volume of the cast iron i. e. the phenomenon of the so-called "growth" of the cast iron takes place. Numerous investigations have been made to prevent such a growth. This applicant noticed that this expansion of the volume of cast iron is caused by the fact that it becomes porous when it is repeatedly subjected to annealing. He performed a series of experiments to make oil permeable cast irons by repeatedly applying annealing operations to a raw grey cast iron and impregnating the resulting product, which has adequately expanded, with a suitable lubricant.

In these experiments, grey iron (specific gravity 7.2) containing:

|                   | Per cent |
|-------------------|----------|
| Carbon (in total) | 3.20     |
| Combined carbon   | 0.50     |
| Silicon           | 2.00     |
| Sulphur           | 0.07     |
| Phosphorus        | 0.70     |
| Manganese         | 0.80     |

was heated to 700° C. and maintained at this temperature for about three hours, and thereafter it was cooled slowly to room temperature. This heat treatment procedure was repeated thirty times. The resulting product was a porous material having a specific gravity of 5.7. It was then immersed into a lubricating oil bath heated to 120° C., whereby a raw cast iron containing 26% of lubricating oil by volume was obtained. The bearing made from this final product by machining proved to be a very satisfactory one as a main bearing of a grinding machine with a main shaft revolving at a speed of 1500 R. P. M., the porosity of the machined bearing surface thereof being seemingly not impaired at all. Indeed, oilless bearings made of this oil permeable cast iron obtained from grey cast iron as set forth previously have been used in practice with a favourable comment.

Since it seems that the formation of iron oxides around graphite-flakes distributed in the mass of a cast iron subjected to repeated annealing is one of causes of the growth of cast iron, this applicant arrived at the conclusion that the porosity of cast iron might be increased,

## 2

if such iron oxides were removed therefrom. Thus, the same raw grey cast iron as used in the previous experiments was heated to 700° C., maintained at that temperature for about three hours and thereafter cooled slowly to ordinary temperature. This procedure was repeated fifty times. The porous cast iron thus obtained, which had a specific gravity of 5.506, was immersed in a bath of 0.25% sulphuric acid solution at room temperature for about 24 hours, and then thoroughly washed with water and completely dried. Its specific gravity then was 5.439. When a circular disc made of this product 30.2 mm. in diameter and 10.2 mm. in thickness was immersed in a bath of lubricant, the quantity of lubricant impregnated in it was 1.666 gr., whereas the quantity of lubricant impregnated in a disc having the same size, but not subjected to said acid pickling treatment proved to be only 1.00 gr. It is thus ascertained that the pickling treatment does increase the porosity of cast iron which confirms the truth of the applicant's aforementioned conclusion. The results of this investigation have already been published.

Through a series of investigations just mentioned, this applicant has recently succeeded in obtaining excellent results in that an oil permeable cast iron having a still much greater mechanical strength can be obtained, and the experimental investigation in the direction of definitely increasing the porosity of the material without appreciably decreasing its mechanical strength has been advanced.

The latest investigations of the oilless bearing, the most important intended field of use of oil permeable cast iron, tends to be directed towards the enhancement of the mechanical strength of the latter, in order to meet the requirements of large type or heavy duty bearings. Consequently, this applicant has further carried out a similar experimental investigation with ferrous materials other than grey cast iron for the purpose of the enhancement of their mechanical strengths. He has found out that when a white pig iron is annealed so as to produce a black heart malleable casting, the structure of the latter will become such that its free carbon is distributed in the matrix of the iron, and that when such a malleable casting is repeatedly heated and cooled, there will be obtained a porous material which is more homogenous than grey cast iron and its mechanical strength is surprisingly increased. Thus a white pig iron (tensile strength 29.8 kg./mm.<sup>2</sup>, Brinell hardness 315 and specific gravity 7.69), having the composition of:

|            | Per cent |
|------------|----------|
| Carbon     | 2.48     |
| Silicon    | 0.92     |
| Manganese  | 0.34     |
| Phosphorus | 0.11     |
| Sulphur    | 0.09     |
| Chromium   | 0.03     |
| Copper     | 0.41     |

and, having been annealed at about 850° C. for twenty-six hours, was heated to a temperature somewhat above or below the A<sub>1</sub> transformation point, that is, 800° C., and then cooled to atmospheric temperature repeatedly, the number of repetitions being fifty times, whereby its mechanical properties became such that its tensile strength was 27.2 kg./mm.<sup>2</sup>, Brinell hardness 80, and specific gravity 7.1. Upon impregnating the material thus obtained with lubricant, it was found that it could contain 4% by volume of the lubricant. Since with grey cast iron after the growth the mechanical strength is at most 13–15 kg./mm.<sup>2</sup>, it is apparent from these results that with white pig iron having a mechanical strength of the order of 27 kg./mm.<sup>2</sup>, a mechanical strength of at least twice that of grey cast iron is readily obtained.

Promoting the investigation for the purpose of provid-

ing a porous, oil permeable cast iron material having a still greater mechanical strength in this way, this applicant has found out that a cast iron which has been caused to have a spheroidal graphitic structure has a greater tensile strength than usual. In consequence thereof, this applicant has succeeded, by heating and cooling such cast iron above and below its  $A_1$  transformation point repeatedly to effect the growth thereof, to obtain a porous, oil permeable cast iron having a mechanical strength three to four times as great as that of an ordinary grey cast iron, and yet capable of absorbing substantially the same amount of lubricant as that absorbed by the latter. In this experiment, a nodular cast iron (tensile strength 60.4 kg./mm.<sup>2</sup>, Vicker's hardness number 290, specific gravity 7.3) containing 0.3% magnesium which was added thereto by employing 80:20 nickel-magnesium alloy and 0.5% silicon added thereto as an inoculant, was repeatedly heated and cooled between a temperature somewhat above or below 800° C. and ordinary temperature, the number of repetition being fifty times, thereby producing a grown up material having a tensile strength of 54 kg./mm.<sup>2</sup>, Vicker's hardness number of 180, and specific gravity of 6.6, which grown up material when subjected to an oil impregnating treatment was capable of absorbing 6% by volume (0.75% by weight) of lubricant. This material is found to be suitable for use in heavy duty oilless bearings.

Based on the results of the aforementioned experiment, and having ascertained that the degree of porosity of a cast iron can be enhanced by repeatedly annealing it to produce a very porous cast iron and then immersing this porous cast iron into a bath of sulphuric acid solution so as to eliminate the iron oxides distributed in that cast iron, this applicant hit on the idea that it would be possible to increase the porosity of a cast iron without sacrificing its mechanical strength, if the cast iron could be converted into one having a small specific gravity by repeatedly subjecting it to annealing operations to produce, in the first place, a porous cast iron having a great amount of iron oxides formed therein, and then reducing said iron oxides to metallic iron. Thus, a porous grey cast iron material (a rod of 30 mm. diameter, 200 mm. long, specific gravity 5.7) obtained from the previous experimental investigation but not yet subjected to said oil impregnating treatment, was exposed to air at ordinary temperature for sixty days. As it was observed that reddish rust of iron oxides had been formed throughout the mass of this material, the latter was subjected to the reduction treatment in a reducing gas stream at a temperature of 700° C. to 800° C. made from cokes. Then it was found that these iron oxides had been definitely reduced and the porosity greatly increased. It thus became apparent from this experiment that prior to the reduction treatment according to the procedure of this invention, the oil containing capacity of the cast iron material was 0.5% by weight, whereas that of the same cast iron after said treatment was 2.5% by weight, that is, its oil containing capacity was multiplied five times. Furthermore, the results of tests of the porous cast iron material thus obtained show that its mechanical strength was by no means reduced at all.

I claim:

1. The method of manufacturing porous cast iron comprising repeatedly heating cast iron to the temperature of its  $A_1$  transformation point and cooling the cast iron to the ambient room temperature, exposing the porous product so obtained to the oxidizing action of air at the ambient room temperature for an extended period of time, and reducing the oxides of the product in a stream of reducing gas.
2. The method according to claim 1 in which the heating and cooling is repeated fifty times from the high temperature of substantially 800° C. to the low temperature of the ambient room atmosphere, the exposure is for a time of the order of sixty days, and the reduction is at a temperature in the range from 700° to 800° C.
3. The method of manufacturing oil impregnated grey cast iron comprising heating the grey cast iron to about 700° C., maintaining the heating for substantially three hours, cooling the grey cast iron slowly to room temperature, repeating said heating, maintaining and cooling at least thirty times, exposing the iron to the ambient atmosphere and temperature for a period of substantially sixty days, subjecting the iron to an oxide reducing gas stream at a temperature in the range of from 700° to 800° C., and immersing the iron in lubricating oil until substantially no further oil is absorbed by the iron.
4. The method according to claim 3 in which the repetition of the heating, maintaining and cooling steps is of the order of fifty times.
5. The method of manufacturing oil impregnated white pig iron comprising heating the white pig iron to a temperature substantially equal to that of its  $A_1$  transformation point, cooling the white pig iron to atmospheric temperature, repeating the said heating and cooling fifty times, exposing the iron to the ambient atmosphere and temperature for an extended period, subjecting the iron to an oxide reducing gas stream, and impregnating the iron with oil.
6. The method of manufacturing oil impregnated nodular cast iron containing 0.3% magnesium and 0.5% silicon comprising heating the nodular cast iron to a temperature of substantially 800° C., cooling the nodular cast iron to room temperature, repeating said heating and cooling substantially fifty times, exposing the nodular cast iron to the oxidizing action of the atmosphere at ordinary temperature for an extended period, subjecting the repeatedly heated and cooled, and exposed nodular cast iron to an oxide reducing gas stream, and then impregnating the nodular cast iron with oil.

#### References Cited in the file of this patent

#### UNITED STATES PATENTS

|           |       |               |
|-----------|-------|---------------|
| 1,511,063 | Pack  | Oct. 7, 1924  |
| 2,187,589 | Lenel | Jan. 16, 1940 |

#### OTHER REFERENCES

"Steel and Its Heat Treatment" by Bullens, vol. 2, 5th ed., 1948, page 255.